

Patented Feb. 15, 1927.

1,617,375

# UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS.

## SHOE STIFFENER.

No Drawing.

Application filed October 31, 1922. Serial No. 598,216.

This invention has relation to stiffeners for footwear, such for example as box-toe or counter stiffeners, and to the sheet material from which the stiffeners are formed.

5 One of the objects of the present invention is to provide a stiffener which may be easily produced by the usual molding operation and which is waterproof and highly water-resistant.

10 In the manufacture of footwear, wherein a molded leather or fiber board counter is employed, it has been customary to temper the molded counter with water so that the heel-seat flange may be softened and caused 15 to conform to the heel-seat in the shoe-making operation. It is desirable, however, that counter stiffeners should be waterproof, and I have discovered that it is possible to produce a molded counter stiffener, the main 20 body of which is waterproof but the skived edges of which may be softened and tempered by the addition of water thereto so as to facilitate the formation of the shoe and yet provide one in which the counter is 25 unaffected by moisture.

Still another object of the present invention is the utilization of the waste material of stiffened box-toe material.

Usually, in the formation of stiffened box-toe blanks, it is customary to saturate sheets 30 of cotton and wool felt with such gums as copal, sandarac, rosin, asphaltum, Montan wax and various other forms of solid hydrocarbons, (either alone or in various combinations) which impart stiffness to the blank and which are easily softened or fused by 35 the application of moderate heat. From sheets thus produced, box-toe blanks are cut, and consequently there is a large amount 40 of waste hydrocarbon-impregnated felt, for which heretofore no use has been found; so that a further object of this invention is to utilize this waste material in the formation of shoe stiffeners.

45 I have found that it is possible to grind this waste box-toe material so as to produce a fibrous mass containing the gums or stiffening agent in a state of fine subdivision. This may be accomplished in an Abbe grinding machine, to which from time to time a 50 small amount of talc may be added to prevent the knives or cutters from being coated with the waterproof gums. It is not possible to introduce the waste material directly

to a beater engine, as the gums which are 55 contained therein are water-repellent and will not disintegrate in the beater in the presence of water, but, by grinding the box-toe waste while dry in an Abbe grinder or other suitable form of grinding apparatus, 60 it is possible to disintegrate the fibrous material sufficiently and to release the gums so that they may be utilized in the formation of the new articles of manufacture. Frequently such box-toe waste contains 80% 65 by weight of the stiffening agent, all of which serves in the formation of a shoe stiffener according to the present invention.

I will now describe one example that is 70 illustrative of the procedure which may be followed in producing shoe stiffener board and of the ingredients which may be utilized in the formation thereof, but it will be understood that I am not limited to the details 75 which I shall describe.

After grinding the waste box-toe material as previously described, so that it is in a state of relatively fine subdivision, 40 parts by weight of such waste and 60 parts by weight 80 of sulphate pulp (or other suitable paper-making fiber) are introduced into a beater with sufficient water to ensure proper circulation of the stock. With the beater roll adjusted to the bed plate, this stock is beaten hard for at least 7 or 8 hours until a very 85 slow and highly hydrated stock is produced. I then add to the beater any suitable material for softening or tempering the gums or other stiffening agent which was added with the waste material to the beater in order that the final shoe stiffeners may have sufficient flexibility to bend or fold without 90 breaking or cracking. In the example now given, I introduce 10 parts by weight of common soap in the form of an aqueous 95 soap solution, which, when precipitated as aluminum soap, will serve the desired purpose. It is desirable also to fix the gums, which are added with the box-toe waste, upon the fibers of the stock, and for this purpose I also add 5 parts by weight of 100 rosin size, and then, after the soap solution and the rosin size are thoroughly beaten into and incorporated in the fibrous stock, I add a precipitating agent such as alum which 105 has the effect of precipitating aluminum soap and aluminum resinate which carry with them and fix upon the fibers the free par-

ticles of gum which were added with the box-toe waste.

The stock, as now prepared, is ready to be formed into sheets. This is accomplished by the use of any well known type of cylinder or wet machine which forms a sheet of fiber board of any desired caliper and size. The sheets thus formed are removed from the make-up roll and dried. In this condition the sheet is relatively dense, but, inasmuch as the gums and the precipitate are distributed in fine particles throughout the sheet, the sheet may be tempered with water so as to render it flexible. In the event that it is desired to provide, for example, a counter stiffener, the body of which is waterproof and the skived edges which form the heel-seat flange are capable of being tempered with water, the counter stiffener blanks are now cut from the sheet and are passed between cylindrical calender rolls which are heated to a temperature sufficient to flux and cause the coalescence of the gums which are incorporated in the sheet. When this is done, the main body of the sheet, which is of the same thickness throughout, is compressed, and becomes waterproof by the fluxing and coalescence of the contained gums, leaving the thinner skived edges porous, uncompacted and uncondensed and with practically no fluxing of the contained gums. The blanks thus formed may now have their skived edges tempered with water and then molded while cold in the usual counter-molding machine. During the tempering operation, the water penetrates only the skived edges of the blanks and does not extend into the main body of the blanks.

It is not necessary, however, that the blanks should be cut from the sheet so as to leave edges which are capable of being tempered with water, although, as stated, for some purposes this is highly desirable. The sheet, after being dried, may be passed as a whole through the heated calendering rolls so that the entire sheet is condensed and compacted and the gums therein fluxed and caused to coalesce. When in this condition, the counter-stiffener blanks may be cut therefrom, and they may be softened by heat to permit their being molded by the usual molding machine, or, if desired, they may be assembled with the upper and heated sufficiently to cause them to become limp and flexible, and then molded to conform to the end of the last during the usual lasting operations.

As further illustrating the procedure which may be followed and as showing that other materials than those herein referred to may be utilized, I may give the following examples in which animal matter while in a gelatinous mass is precipitated on the fibers. In this case, I may use such animal matter as leather, hair, or both, treated with caustic soda to form a gelatinous or col-

oidal solution. For example, 20 parts by weight of scrap leather and 10 parts by weight of cattle hair are treated with a caustic soda solution containing 6 parts by weight of caustic soda until a gelatinous mass is obtained. The beater is furnished with 60 parts by weight of sulphate or other pulp such as utilized in paper manufacture, and, after it has been beaten hard until the stock is slow and thoroughly hydrated, I add the gelatinous mass obtained as previously described. Or, if desired, the hair and leather and caustic soda may be introduced into the beater at the same time as the fiber so that the gelatinous mass is produced during the beating out of the wood pulp. For the precipitation of the gelatinous mass, I now add 10 parts by weight of aluminum sulphate which has the effect of precipitating a gelatinous hydrate intimately mixed with and precipitated on the fibers of the pulp. Then, for the utilization of the box-toe waste previously described, I add 20 parts by weight of such waste after it has been disintegrated in the manner previously referred to. This is thoroughly beaten into the pulpy mass together with 10 parts by weight of finely divided Montan wax until the mass is practically physically homogeneous. I now add an additional amount of alum, say 5 parts by weight, which assists in precipitating and fixing the gums and the Montan wax upon the fibers. If it be desired to color the sheet, any suitable pigment may be added at the same time that the Montan wax is added. For example, I have used 4 parts by weight of red iron oxide or lamp black, and have used aniline dyes in suitable proportion.

The stock is now formed into sheets according to the procedure previously described, and from the dried sheet material the blanks may be cut, skived and calendered, or the sheet itself may be calendered and the blanks then cut therefrom and skived. In either event, after the blanks have been molded into counter stiffeners, they have the appearance and finish of counters made of sole leather. They differ therefrom in the respect that the body portions thereof are waterproof and are not affected by moisture from the foot. A counter stiffener, produced according to the second example, has a further advantage in that it is resistant to oils. Frequently in the manufacture of shoes, the leather employed in making the upper contains oils or greases which would act upon asphalts or gums employed in impregnating felt according to the usual procedure; but, by incorporating in the sheet material the gelatinous precipitate obtained from animal matter treated with caustic soda, the sheet and stiffener blanks cut therefrom are rendered immune to the action of such oils and

greases as are contained in the upper leather so far as softening the blanks is concerned. This gelatinous matter serves excellently as a stiffening agent to keep the main body of 5 the counter stiffener in a firm stiff resilient condition.

What I claim is:—

1. In the manufacture of shoe stiffeners adapted to be softened by the application of 10 heat, the grinding, while in a dry state, of waste fibrous scrap containing a thermo-plastic stiffening agent, until it is finely divided, beating such disintegrated waste together with other fibrous stock, additional 15 thermoplastic agent and water, then sheeting the resultant pulpy mass with the thermo-plastic stiffening agent, in finely divided condition, distributed throughout the sheet, and then forming shoe-stiffener blanks 20 from the sheet.
2. In the manufacture of shoe stiffeners adapted to be softened by the application of heat, grinding dry waste fibrous scrap containing a thermo-plastic stiffening agent, 25 pulping such ground waste together with fibrous stock and additional thermoplastic agent in water, fixing the particles of thermo-plastic agent on said fibers, then sheeting the pulpy mass on a paper machine, and then cutting shoe-stiffener blanks 30 of appropriate size and shape from the sheet.
3. In the manufacture of shoe stiffeners adapted to be softened by the application 35 of heat, grinding dry waste fibrous scrap containing a thermo-plastic stiffening agent, pulping such ground waste together with fibrous stock in water, incorporating in the mass a material for softening the thermo-plastic stiffening agent, fixing the particles 40 of said stiffening agent on the fibers by a precipitate, then forming the pulpy mass into a sheet, and then cutting shoe-stiffener blanks 45 of appropriate size and shape from the sheet.
4. In the manufacture of shoe stiffeners adapted to be softened by the application of heat, grinding dry waste fibrous scrap containing a thermo-plastic stiffening agent, 50 pulping such ground waste together with fibrous stock in water, incorporating in the mass a material for softening the thermo-plastic stiffening agent, fixing the particles of said stiffening agent on the fibers by precipitating a size in the pulpy mass, then 55 forming said mass into a sheet on a paper machine, and then cutting shoe-stiffener blanks of appropriate size and shape from the sheet.
6. In the manufacture of shoe-stiffeners adapted to be softened by the application of heat, grinding waste fibrous material containing a thermo-plastic stiffening compound, pulping such disintegrated material together with paper-making fibrous material and a finely divided thermo-plastic compound, fixing the thermo-plastic compounds on said fibers, forming the resultant 70 pulpy mass into a sheet, and then cutting shoe-stiffener blanks from the sheet.
7. In the manufacture of shoe-stiffeners adapted to be softened by the application of heat, grinding waste fibrous material containing a thermo-plastic stiffening compound, pulping such disintegrated material together with paper-making fibrous material and finely divided Montan wax, fixing the particles of said thermo-plastic compound 75 and said Montan wax on the fibers of the pulp, sheeting the resulting mass, and then cutting shoe-stiffener blanks from the sheet.
8. In the manufacture of shoe stiffeners adapted to be softened by the application of 80 heat, grinding waste fibrous material containing a thermo-plastic stiffening compound, pulping such disintegrated material together with paper-making fibrous material and a finely divided thermo-plastic compound, fixing said thermo-plastic compounds on the fibers by the precipitation of a gelatinous precipitate, forming the mass into a sheet, and then cutting shoe-stiffener blanks 85 from the sheet.
9. In the manufacture of shoe stiffeners adapted to be softened by the application of heat, grinding waste fibrous material containing a thermo-plastic stiffening compound, pulping such disintegrated material 90 together with papermaking fibrous material and a finely divided thermo-plastic compound, fixing said thermo-plastic compounds on the fibers by the precipitation of a gelatinous precipitate, forming the mass into a sheet, and then cutting shoe-stiffener blanks 95 from the sheet.
10. In the manufacture of shoe stiffeners adapted to be softened by the application of heat, beating cellulosic stock with water until the same is well hydrated, mixing there- 100 with a gelatinous animal matter, precipitating a gelatinous hydrate by the addition of a precipitate, mixing disintegrated waste fibrous material containing a thermo-plastic compound with the pulpy mass together with finely divided Montan wax, mixing a precipitating agent into the said mass, 105
11. In the manufacture of shoe stiffeners adapted to be softened by the application of heat, grinding dry waste fibrous scrap containing a thermo-plastic stiffening agent, 110 pulping such ground waste together with fibrous stock in water, incorporating in the mass a material for softening the thermo-plastic stiffening agent, fixing the particles of said stiffening agent on the fibers by precipitating a size in the pulpy mass, then 115 forming said mass into a sheet on a paper machine, and then cutting shoe-stiffener blanks from the sheet.
12. In the manufacture of shoe stiffeners adapted to be softened by the application of heat, beating cellulosic stock with water until the same is well hydrated, mixing there- 120 with a gelatinous animal matter, precipitating a gelatinous hydrate by the addition of a precipitate, mixing disintegrated waste fibrous material containing a thermo-plastic compound with the pulpy mass together with finely divided Montan wax, mixing a precipitating agent into the said mass, 125
13. In the manufacture of shoe stiffeners adapted to be softened by the application of heat, grinding dry waste fibrous scrap containing a thermo-plastic stiffening agent, 130 pulping such ground waste together with fibrous stock in water, incorporating a sapon-

finally forming said mass into a sheet, and then cutting shoe-stiffener blanks from the sheet.

11. In the manufacture of shoe stiffeners, forming an aqueous pulp of fibers, a finely divided thermo-plastic material, and a precipitate by which the particles of thermo-plastic material are fixed upon the fibers, forming such pulp into a porous sheet and drying the same, cutting shoe stiffener blanks from such sheet, skiving such blanks, and heating and compressing the unskived portions of the blanks to cause a coalescence of the thermoplastic particles therein, where by the body portions of such blanks are substantially non-absorbent, and the skived edges are water-absorbent but may be rendered water-repellent on being subjected to heat and pressure.

12. A shoe stiffener comprising a water-resistant body portion, and having edge portions which may be softened by the application of water.

13. A molded shoe stiffener comprising

a stiff water-resistant body portion and a porous skived edge portion adapted to be made water-resistant on the application of heat and pressure.

14. A molded shoe stiffener of appropriate shape and having a body comprising fibrous material, and a thermo-plastic material and a precipitate both distributed throughout the fibrous material, said stiffener being water-repellent and being adapted to be softened by the application of heat.

15. A molded felted fibrous shoe stiffener of appropriate shape and having a body adapted to be softened by the application of heat, comprising fibrous shoe-stiffener waste containing a thermo-plastic compound, 40 cellulosic fibers and a precipitate, all in intimate mixture, the precipitate acting to fix the thermo-plastic content of said waste upon the fibers.

In testimony whereof I have affixed my 45 signature.

ALBERT L. CLAPP.